

# UNITED STATES PATENT OFFICE.

RALPH H. MCKEE, OF NEW YORK, N. Y., AND ANDREW A. HOLMES, OF BOSTON,  
MASSACHUSETTS.

## PROCESS OF MAKING PAPER-PULP.

1,360,658.

Specification of Letters Patent. Patented Nov. 30, 1920.

No Drawing.

Application filed May 24, 1919. Serial No. 299,632

To all whom it may concern:

Be it known that we, RALPH H. MCKEE and ANDREW A. HOLMES, citizens of the United States, residing at New York and Boston, in the counties of New York and Suffolk and States of New York and Massachusetts, respectively, have invented certain new and useful Improvements in Processes of Making Paper-Pulp, of which the following is a specification.

This invention relates to a process of making paper pulp and has particular reference to an improved process of this character which is adapted to produce pulp from resinous woods, which is sufficiently free from resin to enable it to be used in making paper of a high grade.

For many purposes the sulfite process of making paper pulp gives the best type of paper pulp. However, by the methods hitherto known resinous woods (*e. g.* southern pines) do not yield to the sulfite process to give a pulp sufficiently free from resin to make a paper of good quality for most purposes, *e. g.*, a bond writing paper. Such woods are commercially only used for the manufacture of sulfate or soda pulp, *i. e.*, for pulp useful for wrapping paper or soft book paper, or the like.

We have discovered that when chips of such a resinous wood are extracted with a resin-dissolving solvent and the solvent removed, the remaining wood chips when subjected to the customary sulfite pulp treatment give a paper pulp which in quality compares favorably with the standard pulp made by the sulfite process from non-resinous woods, such as spruce.

As a solvent, any of the resin-dissolving solvents such as benzol or carbon bisulfid may be used, but we prefer to use liquid sulfur dioxid. In case such a solvent as benzol or carbon bisulfid is used, the wood chips after extraction are steamed to remove and recover the remaining portion of the solvent and then sent to the digester where they are "cooked" by the customary methods used to produce soda, sulfate or sulfite pulp. Liquid sulfur dioxid has the advantage over solvents previously mentioned that it carries no fire risk, is much more cheaply produced, and the portion remaining in the chips after extraction need not be removed before the next step of cooking to a pulp when the sulfite process is

used. In fact, this residual sulfur dioxid remaining in the chips is a distinct advantage in the succeeding step of sulfite pulp manufacture.

Liquid sulfur dioxid has the disadvantage that it vaporizes at ordinary pressure and consequently must be used under a pressure sufficient to keep it liquid during the time it is being used to remove the resins from the chips. Distillation of the solvent from the resulting solution leaves the extractable material behind. This can then be prepared for the market by the customary methods of the art.

When sulfur dioxid is the solvent used, we prefer, although this is not a necessary procedure, to extract in the same vessel as that in which the succeeding step of cooking with sulfite "acid" is next carried out, *i. e.*, to use the sulfite digester for the extraction as well as for the cooking to pulp.

Our process will be more clearly understood from the following example illustrating our preferred procedure.

Bark and chip the long leaf pine (*Pinus Australis*) from which the pulp is to be made and dry the chips below 20 per cent. moisture. This drying is not essential but is desirable as it shortens the period of extraction and has other desirable features.

Then fill the digester with the chips and produce a partial vacuum in the digester so as to remove the larger part of the air present around and within the chips. This withdrawal of air is not essential to the process but serves to hasten the extraction and to reduce the amount of relief gases that have to be handled during the extraction process.

Sulfur dioxid in liquefied form and preferably at a somewhat elevated temperature, say one giving a pressure of 75 pounds per square inch gage pressure, is then passed into the chips. This liquid is kept in contact with the chips for a length of time, which depends on the size of the chips. It is then pumped off and fresh sulfur dioxid introduced to complete the extraction. If necessary to remove the greater part or if desired, substantially all of the resin, a third charge of sulfur dioxid may be used but two are ordinarily sufficient. The relief gases, if any, are piped to the acid making plant for strengthening the cooking acid.

The resulting solution of the rosin, tur-

pentine and small amounts of other extractives in liquid sulfur dioxid is then distilled in such a manner that the sulfur dioxid is recovered in liquid form for reuse, preferably being distilled under pressure. The residue consisting of rosin, turpentine, etc., and a little dissolved sulfur dioxid is then placed in a second still and distilled in such a manner as to separate the sulfur dioxid from the turpentine and leave the residue of molten rosin in the still. The molten rosin is drawn off into barrels and is ready for the market. The turpentine so produced is for many purposes satisfactory, but in other cases it can with advantage be subject to further refining, *e. g.*, washing with alkali and redistilling. The gas which contains sulfur dioxid, escaping from the stills is sent to the "acid making" plant of the sulfite pulp department to be used for strengthening the cooking acid.

The chips in the digester which have had the rosin and turpentine largely removed by the extraction effect of the liquid sulfur dioxid are now covered by the customary cooking acid used in the sulfite pulp industry except that this acid may be of less than the customary strength to the extent of the amount of the sulfur dioxid remaining in the chips. The "customary cooking acid" to which reference is made consists of a water solution containing approximately one per cent. of sulfur dioxid combined with lime (calculated as  $\text{CaSO}_3$ ) and four per cent. free sulfur dioxid, largely in the form of sulfurous acid ( $\text{H}_2\text{SO}_3$ ).

Steam is turned on and the sulfite cooking process is carried out in the customary manner, seven to eleven hours time being required according to the character of paper to be made.

The resulting pulp is washed and bleached in the customary manner and is ready for the manufacture of paper. Recoveries of the sulfur dioxid in the escaping gases are made in the customary manner.

The residual waste sulfite liquor can be used for the making of alcohol, etc., as described in the Letters Patent Nos. 1,273,392, 50 1,284,739 and 1,284,740 by one of us.

While for the purpose of illustration we have described in detail the preferred practice of our process, it is to be understood that the details of procedure may be widely varied without departing from the spirit of 55 our invention or the scope of the subjoined claims.

Having described our invention, we claim:

1. The process of making paper pulp consisting in first subjecting resin containing wood to the action of liquid sulfur dioxid and then to the action of a pulp producing operation whereby paper pulp is produced therefrom. 60

2. The process of making paper pulp 65 consisting in first subjecting resin containing wood to the action of liquid sulfur dioxid at an elevated temperature and at superatmospheric pressure and then to the action of a pulp producing operation whereby paper pulp is produced therefrom. 70

3. The process of making paper pulp consisting in first subjecting resin containing wood to the action of liquid sulfur dioxid and then to the action of the sulfite process 75 whereby paper pulp is produced therefrom.

4. The process of making paper pulp consisting in first subjecting resin containing wood to the action of liquid sulfur dioxid, separating the liquid sulfur dioxid from its 80 dissolved content and subjecting the treated wood to the action of a pulp producing operation whereby paper pulp is produced therefrom.

5. The process of producing paper pulp 85 from resin containing wood which consists in placing the wood in a sulfite digester, subjecting it to the action of liquid sulfur dioxid, removing the main portion of the sulfur dioxid from the digester, adding sulfite 90 liquid and subjecting the treated wood to the sulfite cooking process whereby paper pulp is produced therefrom.

In testimony whereof we affix our signatures in presence of two witnesses.

RALPH H. MCKEE.  
ANDREW A. HOLMES.

Witnesses:

L. V. EATON,  
M. B. McDONALD.